

June 6, 1933.

G. Mack. BROWN

1,912,885

METHOD OF COATING

Filed Feb. 13, 1930

2 Sheets-Sheet 1

Fig.1.



Fig.2.



June 6, 1933.

**G. MacK. BROWN**

1,912,885

### METHOD OF COATING

Filed Feb. 13, 1930

2 Sheets-Sheet 2



**INVENTOR**

George M. Brown.  
by

Bynes, Stebbins, Parmelee & Blenko  
Atty's.

## UNITED STATES PATENT OFFICE

GEORGE MACKENZIE BROWN, OF LONDON, ENGLAND

## METHOD OF COATING

Application filed February 13, 1930, Serial No. 428,138, and in Great Britain February 15, 1929.

- This invention comprises improvements in or relating to processes and apparatus for surfacing sheet material with pigments, varnishes, lacquers, waterproofing solutions or the like. The manufacture of "marbled" papers is a good illustration of the application of this invention, the expression "marbled" being used in a broad sense to include papers with ornamental coatings, either monochrome or multicolour, not only in forms or patterns which are more or less imitative of marbles, but also in forms, such as waves, washes or stripes, which may be more or less irregular and may sometimes be substantially uniform. In the known hand process of marbling paper, colour is deposited in a tank or tray on the surface of a liquid medium (e.g. a solution of carragheen moss) upon which it will float, and spreading naturally over the whole of that surface the colour forms a thin cohesive film. More or less irregular patterns may be produced in the film by stirring, and thereafter, on application of a sheet of paper to the surface of the liquid, the film adheres to the paper and is removed from the liquid medium on removal of the sheet.
- The above process is applicable only to the marbling of single sheets, a sheet at a time, and it will be understood that after the removal of the film a new film must be formed on the surface of the flotation liquid. With certain colours and certain flotation media it is possible from a single film to coat two or even three or four sheets, but the coatings on the subsequent sheets are thinner than and inferior to that on the first sheet. In any case this hand marbling process is necessarily laborious and costly.
- One object of the present invention is to provide an improved and inexpensive process which can be carried out mechanically and continuously for the production of ornamented sheet material, such as marbled paper, in continuous lengths, or in a succession of single sheets, giving effects such as have previously been referred to as "marbled" effects as well as coatings of colour which may be flat or almost flat.
- This invention is based on the fact that films produced by the deposition on a flotation medium of suitable liquid compositions have sufficient tensile strength to enable them to be drawn along the surface of the flotation liquid without disruption.
- The suitable liquid composition may comprise pigments in vehicles or media, such as boiled linseed oil, and/or cellulosic solutions (e.g. a solution of a cellulose ester or ether). The composition may also include thinning agents and/or volatile solvents. Instead of or in addition to pigments, the composition may comprise varnishes, lacquers, waterproofing solutions and dyes.
- The process according to this invention comprises the step of traversing a film-receiving surface past a fixed station over a tray, trough or the like containing the liquid medium on which the film is carried, in such manner that successive portions in the length of the film-receiving surface come into contact with the liquid at the station and remove the film by drawing it along the surface of the liquid to the station while the body of the liquid remains substantially stationary.
- It has hitherto been proposed (see for example British specification No. 130,883) to carry out mechanically a marbling process by traversing a continuous web of paper over the surface of a marbling liquid contained in a trough in such manner that successive portions in the length of the web come into contact with the liquid at successive points along the length of the trough. In such a process, which necessitates complicated apparatus (e.g. an annular trough rotatable bodily or a web-carrying cylinder movable bodily round the trough), the pigment is picked up by what is in effect a rolling motion of the receiving surface in relation to

that of the marbling liquid. A similar effect is also obtained in another known process in which, e. g. by creating a current in the floatation liquid, that liquid is moved bodily with the film on it up to a station at which the film is taken off by the paper. The process according to the present invention depends upon a different effect, namely, the drawing of a film along the surface of the floatation medium, the body of the latter remaining substantially stationary.

One example of apparatus which may be employed in the carrying out of this invention will now be described with reference to the accompanying drawings (to some extent diagrammatic) in which—

Figure 1 is a side elevation of the machine taken at the line 1—1 in Figure 2.

Figure 2 is a (shortened) plan of the machine shown in Figure 1, and

Figure 3 is an end elevation of the machine.

Like reference numerals indicate like parts throughout the figures.

In the apparatus illustrated the film is formed on the surface of a liquid floatation medium contained in a tray 10. The paper 11 to be coated is mounted on a reel 12 supported above the tray. From this reel the paper is drawn off and passed over a guide roller 13 and then under a doctor 14 which dips into the liquid in the tray 10 to a depth of about a quarter of an inch. In this example the doctor is a flat blade; it may in other cases be constituted by a roller. After passing under the blade 14 the paper is taken over a guide roller 15 and is then wound on to a reel 16. The blade 14 is located near the back of the tray 10 while near the front thereof the paint or other film-forming material is deposited on the floatation medium from pots or droppers 17 mounted on a bar 18. Each of the droppers 17 (of which any desired number may be provided) has a tapered nozzle the outlet from which is controlled by a needle valve 39 adjustable at will. The droppers 17 are adjustable along the bar 18 to any desired settings. Between the dropper bar 18 and the blade 14 there is located a mechanical agitator comprising a shaft 19 on which is mounted a series of inclined discs 20 so arranged that adjacent discs are at opposite inclinations to the axis of the shaft. The shaft 19 is continuously rotated by a chain drive 21 from a power-driven shaft 22 on which the take-on reel 16 is mounted. The dropper bar 18 is continuously reciprocated, in a direction transverse to the travel of the paper, by means of a crank 23 and connecting rod 24, the crank being on a shaft 25 gear driven from a power shaft 26.

In the operation of this apparatus, the paint or like film-forming liquid is supplied continuously at the front of the tray 10, and

at the back of the tray the paper web is continuously traversed through the floatation medium. The liquid delivered from the droppers 17 spreads out naturally over the surface of the floatation medium and forms a thin cohesive film. The reciprocation of the dropper bar 18 ensures the required distribution of the paint over the surface of the floatation medium. Between the region at which the paint is supplied and the region at which the paper is traversed through the tray, the film is agitated by the discs 20 which produce a wave-form effect. It will be seen therefore that in the operation of this apparatus there is a continuous formation of film which is drawn off along the surface of the floatation medium on to the paper web, with substantially no agitation of the body of the medium.

The movement of the web may exert a certain slight dragging action on the floatation medium and this may tend to set up return currents which may interfere with the formation and distribution of the film. In order to avoid this difficulty a still pool may be formed in the tray 10 by immersing to a slight depth in the floatation medium an open frame 27. As shown in Figure 2 this frame is of about the same width as the blade or doctor 14 and it is of such dimensions that a space is left between the sides of the frame and the adjacent sides of the tray. The paint is dropped into the pool enclosed by the frame, and the space outside the frame allows the floatation medium to recover its level, after the slight displacement caused by the dragging action of the paper, without setting up return currents within the pool.

If desired the agitator shaft 19 in addition to or instead of being rotated, may have imparted to it a reciprocating motion by means of an eccentric 28 on the shaft 26 and a coupling rod 29. The reciprocation of the shaft 19 will not usually be required where the agitators take the form of oblique discs such as 20, but with other forms of agitator reciprocation of the shaft may be desirable. It will be appreciated also that in some cases the agitator may be completely omitted from the apparatus, thus allowing the film to follow its natural course. Alternately a fixed comb or like device, through or past which the film will be drawn, may be provided instead of or in addition to the agitator.

In an alternative form (not illustrated) the paint supply means may comprise large containers in which the paint is agitated mechanically (e. g. by a pump), combined with rubber supply tubes leading from these containers to various points situated above the tray 10. These supply tubes may be arranged to provide either a continuous or an intermittent supply, and they may if desired be furnished with control devices mechanically

operated (e. g. by cams) to regulate the delivery of the paint.

The patterns which are produced on the web 11 by the operation of the apparatus depend upon a number of different factors, for example the nature, and movement, if any, of the paint distributing devices, the distance between the paint distributors and the doctor 14, the particular form of agitator employed 10 and the speed of the motion which is imparted to it, and also the speed at which the paper is run through the machine. As will be appreciated different combinations of these factors produce an indefinite number of different patterns. Straight and uniformly striped patterns may be produced by dropping the colours into parallel compartments leading up to the doctor 14 or equivalent device, and these compartments may for example be formed by strings, strips or the like 20 stretched across the tray 10 so that they are partly immersed in the flotation medium.

If desired the movement of the film towards the point at which it is drawn off by 25 the web, may be accelerated mechanically or by hand.

With the apparatus illustrated herein the supply of the paint and the agitation of the film to form patterns is carried out to a large 30 extent mechanically. It is to be understood that either or both of these operations may be effected by hand, and in some cases e. g. in the imitation of fine marbles, it may be preferable to adopt the hand method.

35 In carrying out the process according to this invention the following film-forming materials have been used successfully (a) printer's ink diluted with petrol (b) Reeves' waterproof poster colours similarly diluted 40 with petrol and (c) cellulose lacquers diluted with thinners. In general the film-forming materials should have the following characteristics. They should, when properly diluted, form fairly thick drops which will 45 not sink but will spread out quickly in a film. They must not mix with the flotation medium and finally they should be such that they will readily adhere to the surface of the article to be coated. In the known hand process for 50 the preparation of marbled papers, ox-gall and "sprinkling water" are used (a) to make the special colours used for hand-marbling float better and (b) to make blobs in the film. These materials may also be employed 55 in carrying out the process according to the present invention. Films of irregular patterns may be produced by depositing the colour on the flotation medium with a spray or by spraying ox-gall, water or other liquids 60 upon the colour.

The flotation medium upon which the film is formed may be an aqueous solution of caragheen moss, or in many cases plain water may be used.

65 According to a further feature of this in-

vention portions of the sheet to be coated are treated with a "resist", prior to the coating operation, so as to prevent the deposition of the film on said portions. The resist may be constituted by any material which will prevent adhesion of the film to the surface of the sheet. In working with certain pigments water and a sugar solution, have been used successfully as resists. It is within the invention to apply a resist of such a nature 70 that it will not entirely prevent the picking up of film by the treated portions, but will only modify the amount of film applied. In other words an imperfect resist may be used. The resist may be applied in any convenient way, for example by means of a roller having a pattern in relief, or by spraying through a stencil. The resist may be printed in ink as a design on the paper, the latter being traversed through the film carrying 75 medium while the ink is still wet.

The invention is applicable not only to the coating of paper but also to the treatment of textile material and sheet material generally. In treating textile material the 80 films may comprise a dye or dyes.

While the process in its preferred form is applied to the production of coated sheet material in continuous lengths, the process may also be used for coating a succession of separate sheets by a continuous operation. In the latter case the sheets may be fed one at a time to grippers on a cylinder which rotates in contact with the marbling liquid, or the sheets may be carried by endless bands 95 or the like which are traversed over the surface of the liquid. While it is preferable that the film should be applied direct to the surface of the paper or other sheet material, it is within the invention to employ a film transfer roller or other intermediate film-receiving surface, which takes off the film from the flotation medium and transfers it to the paper or other material to be treated.

100 The apparatus described herein may be modified in many ways. For example, two webs of paper may be simultaneously marbled from one tray by having pigment supply means at opposite ends of the tray and by drawing off two films at the centre of the tray. Similarly, both sides of a web may be marbled by traversing opposite sides of the web through different trays. Again, a web marbled in one tray may be conducted to another 105 where it will receive a coating of a different pigment.

110 In the appended claims in which is recited "a stationary flotation medium", or the equivalent thereof, such limitation is not to be construed as precluding a local agitation of the 115 color film on the surface of the medium or its movement therealong.

I claim.

1. A method of coating paper including 120 the steps of supplying film-forming liquid

to one region of the surface of a body of a flotation medium which is substantially stationary and undisturbed, except possibly for local agitation or movement of the film on the 5 surface of the liquid, engaging the film with a continuous paper web moving past a region fixed relative to the body of the medium and spaced from the first-mentioned region, pulling the film by its surface tension from the 10 first-mentioned region to the second-mentioned region, and stripping it from the medium at the latter.

2. A method of coating paper including the steps of supplying coating fluid to a flotation medium to form a coating film on the 15 surface thereof, maintaining the body of the medium substantially stationary, and removing the film from the medium by traversing a paper sheet past a fixed point adjacent the liquid surface to pick up the film and draw additional coating material toward said point over the surface of the stationary flotation 20 medium.

3. A method of coating paper including the steps of supplying film-forming fluid to a stationary body of a flotation medium, and removing the film from the medium by continuously bringing paper into engagement 30 with the film at a fixed point to cause adherence of the latter to the former for stripping it from the medium and moving the film across the surface of the medium by its own surface tension.

4. A method of coating sheet material including the steps of forming a coating film on the surface of a body of liquid while maintaining the liquid substantially stationary, and traversing a film-receiving surface past a fixed point near the surface of the liquid 40 to cause adherence of the film to the receiving surface and movement of the film over the surface of the liquid.

5. A method of coating including the steps of supplying film-forming liquid to a stationary flotation medium at one station on the surface thereof, and picking up said film and drawing it along said surface by causing a continuous web to engage the film at another 50 fixed station on said surface.

6. In a method of coating, the steps including supplying a film-forming fluid to a stationary flotation medium, and drawing the film along the surface of the medium and 55 stripping it therefrom by traversing a continuous web past a fixed point, in engagement with the film.

7. A process according to claim 6 including the additional step of treating portions of the 60 web with a "resist" prior to the coating operation, to prevent deposition of film on said portions.

8. A process as claimed in claim 6 including the additional step of effecting local agitation 65 in the film while the latter is being drawn

along the surface of the flotation medium, to form a pattern on the film.

9. A process according to claim 6 including the additional step of depositing the film-forming fluid on the flotation medium so as 70 to make a patterned film.

10. A process according to claim 6 including the additional step of confining the deposition of the film-forming fluid to portions of said medium spaced from the edges 75 thereof.

In testimony whereof I affix my signature.  
GEORGE MACKENZIE BROWN.

80

85

90

95

100

105

110

115

120

125